

Jan. 3, 1939.

C. G. MAIER

2,142,694

PROCESS FOR REDUCING CHROMIUM COMPOUNDS

Filed Aug. 3, 1937



INVENTOR.  
Charles G. Maier  
BY  
Robert N. Eckhoff  
ATTORNEY.

## UNITED STATES PATENT OFFICE

2,142,694

## PROCESS FOR REDUCING CHROMIUM COMPOUNDS

Charles G. Maier, Oakland, Calif., assignor to  
Great Western Electro-Chemical Company, a  
corporation of California

Application August 3, 1937, Serial No. 157,154

17 Claims.

(Cl. 75—84)

This invention relates to a method of reducing a chromium chloride to chromium, and, more particularly, to a method of reducing chromium trichloride with hydrogen to provide chromium and especially chromium as sponge chromium.

*A definition of sponge chromium*

The term "sponge" as applied to a metal has a very definite meaning. The term has been heretofore loosely applied in the art as describing metals heretofore produced by low temperature operations without regard for the actual metal produced. Sponge metals have been properly defined as those reduced, usually by gaseous agents, from oxidic compounds of the metal under such low temperature conditions with respect to the melting point that grain growth, cementation, or incipient fusion of the reduced metal does not take place. The material is thus macroscopically pseudomorphic with the particles of the source material, but under high magnification is seen to consist of aggregates of very minute metallic particles, which in general are of an individual grain size of a micron or less. Since the macroscopic form is preserved, the whole structure is thus cellular or porous, whence the name "sponge" metal is applied.

While sponge iron is so produced commercially, and is a material recognized as having metallurgical advantages for special purposes, sponge chromium has not been produced commercially, nor have previous investigations disclosed a workable method of manufacturing it, despite its obvious interest for use in powder metallurgy.

35 *The prior art*

The reason why sponge chromium can not be prepared by conventional methods, such as are used for iron, resides, I have found, in the exceptionally high stability of chromium oxide ( $\text{Cr}_2\text{O}_3$ ). Usual reducing gases are only very weakly reducing on this oxide even at very high temperatures. Thus, taking the typical example of the reduction of  $\text{Cr}_2\text{O}_3$  by hydrogen, the equilibrium constant for the reaction



is at  $1200^\circ\text{C}$ ,  $1.3 \times 10^{-4}$ ; at  $1400^\circ\text{C}$ ,  $5.5 \times 10^{-4}$ ; and near the melting point of chromium (which has been given at  $1530$ — $1570^\circ\text{C}$ ) about  $1.6 \times 10^{-3}$ . Thus the amount of water vapor produced by passing pure hydrogen at one atmosphere pressure over chromium oxide is at  $1200^\circ\text{C}$ , only .01%; at  $1400^\circ\text{C}$  about .06%, and at the melting point, about 0.16%. This shows the high stability of this oxide.

It has been proposed to reduce chromic oxide by hydrogen at temperatures near  $1500^\circ\text{C}$ , by recirculating hydrogen gas repeatedly (obviously over a thousand cycles would be needed to use it up at  $1500^\circ\text{C}$ ), and each time removing the minute amount of water formed per cycle by freezing it out with liquid air. Such a process I deem uneconomical, and subject to great difficulty in adaptation to commercial use because of the very serious difficulties of finding materials gas tight to hydrogen at these temperatures, as well as to the low cyclic efficiency.

Other investigators have produced what they term as sponge metals, including chromium. However, upon consideration of these, it will be readily seen that they do not have and could not possibly have produced sponge chromium. For example, Flodin in U. S. Patent 1,792,532 of February 17, 1931, produced an alloy of iron and chromium. Flodin first formed an iron-chrome oxide briquet which contained silicon but which he claimed was substantially free of carbon. Thereafter, this briquet was heated to  $1150$ — $1300^\circ\text{C}$ . to the end that the silicon reduced the chromium oxide. Since the material included iron, grain growth necessarily followed, since this begins in iron near  $900^\circ\text{C}$ . It is obvious that Flodin's material could not answer the definition of a substantially pure, true sponge chromium.

It has been proposed to reduce chromic oxide with hydrogen at  $900$ — $1100^\circ\text{C}$ . according to the reaction



See Rich, U. S. Patent 1,741,955. Meyer has (Kaiser Wilhelm Inst. Eisenforsch 13, 1931, p. 199) stated that he could not effect this reduction at  $900^\circ\text{C}$ . In any event, assuming Rich has an operative process, the equilibrium constant for this reaction is  $1.3 \times 10^{-4}$  at  $1200^\circ\text{C}$ . My experimental observations have shown grain growth in chromium to begin below this temperature and to be appreciable at this temperature. From the low equilibrium constant it should be obvious that even at  $1200^\circ\text{C}$ . an enormous hydrogen to oxide ratio must be used. Rohn, in Patent 1,915,243 of June 20, 1933, proposed operation at  $2000^\circ\text{C}$ . Baukloh and Henke (Zeit. fur Anorg. und All. Chemie 237 (1937), 307—310), give the percentages of reduction effected by hydrogen for various temperatures. According to them about eight hours are required at  $1000^\circ\text{C}$ . to effect as much as an 8% reduction and at  $1200^\circ\text{C}$ . only 40% reduction is achieved in this time period.

*The non-equivalence of hydrogen and other reductants*

As will appear hereinafter, I have found that the reduction of chromium chloride to produce sponge chromium must be conducted in a relatively narrow temperature range—between 775–815° C., the upper temperature being that at which chromous chloride melts. Preferably, the reaction is carried out between 775 and 802° C.

10 In Patent 1,373,038, Weber states that chromium chloride can be reduced by metallic iron to metallic chromium over a temperature range between 700 and 1200° C. I have determined that when the reducing agent is not a gaseous medium, 15 a true sponge metal cannot result as a product. In the case of Weber's process, the reducing medium is a metal, particularly iron. Within the temperature range specified by Weber, iron is not a gaseous reducing medium. It should also be 20 particularly noted that the reduction of chromium oxide at temperatures near its melting point causes rapid grain growth in the metal, and such a product could not fall within the proper and accepted definition of a true sponge metal.

25

While carbonaceous reductants, such as carbon monoxide, or methane, are more powerful reducing agents than hydrogen at temperatures above about 900° C., these materials result in the 30 formation of chromium carbide, which renders the product unsuited to the special requirements of powder metallurgy or the manufacture of stainless steels. Hydrogen therefore stands alone as a reducing agent for production of sponge 35 chromium from a chromium chloride.

*General considerations of the process*

I have discovered a method of reducing a chromium bearing material, as CrCl<sub>3</sub>, to metallic 40 chromium at a temperature as low as 780–800° C. by hydrogen gas, and have succeeded in manufacturing a new and desired metallurgical material, sponge chromium of high purity.

My investigations of the reduction of chromous 45 chloride by hydrogen CrCl<sub>2</sub>+H<sub>2</sub>=Cr+2HCl show that the amount of hydrochloric acid in equilibrium with hydrogen (when the total pressure was 1 atmosphere) was at 700° C., 1.05%; at 750° C., 1.87%; at 800° C., 3.12%; and at 815° C., 3.60%. 50 At 815° C., pure chromous chloride melts, and, in the process of melting, easy access of hydrogen is hindered, so that reduction is slow at temperatures in the liquid range; 815° C. at one atmosphere therefore provides a limiting upper 55 temperature.

The first stage of reduction of chromium trichloride is, under normal circumstances, to the dichloride, rather than to metal. The reaction 2CrCl<sub>3</sub>+H<sub>2</sub>=2CrCl<sub>2</sub>+2HCl is substantially irreversible, and for all practical purposes may be considered to go completely to the right, and at equilibrium results in virtually complete usage of the hydrogen. The reaction rate becomes appreciable near 400° C., and near 800° C. is apparently limited only by gaseous diffusion rates in the heterogeneous system.

The direct reduction of CrCl<sub>3</sub> to metal by hydrogen is normally prevented by the dichloride formation. If direct reduction to metal could be obtained I have determined that the following HCl concentrations could be expected, when the total pressure is 1 atmosphere: at 600° C., 10.4% HCl; at 700°, 29.7%; and at 800°, 58.5%.

75 Since, under normal circumstances, chromium

dichloride formation is usually the first step of the reduction, the melting points of mixtures of dichloride and trichloride is further important. Investigation showed that a eutectic is formed between CrCl<sub>2</sub> and CrCl<sub>3</sub> which melts near 802° C., and contains slightly over 4 mol percent of CrCl<sub>3</sub>.

The vapor pressure of chromium trichloride begins to become appreciable at temperatures near 800°. Thus it is .002 atmosphere at 700° C.; .01 at 750°; .04 at 800°; and 0.13 at 850°.

The reduction of chromium trichloride by hydrogen to metal is possible with a theoretical utilization of hydrogen corresponding to the limit set by equilibrium of 3.12% HCl at 800° C., and in a continuous counter-current reduction apparatus 15 the limiting normal HCl content is

$$3.12 \times 1.5 = 4.68\%,$$

corresponding to the stoichiometric relationships Cr:CrCl<sub>2</sub>:CrCl<sub>3</sub>. Any concentration of HCl above 20 3.12% will cause reversal in that part of the reduction unit where the metal is present, but by using a counter-current process I can secure higher HCl concentrations. To avoid fusion and volatilization, and to ensure the macroscopic 25 retention of form required to produce sponge chromium, temperatures above 802° C. should not be utilized, although where sponge chromium is not desired the temperature can vary between 775° C. and 850° C. Above 850° C. the material vaporizes 30 faster than it reduces and difficulties due to vaporization are encountered.

*Hydrogen purification*

Passing commercial hydrogen over the trichloride under these conditions, did indeed produce some chromium metal, but only in a form badly contaminated with oxide. Further, I found that ordinary methods of removing the hydrochloric acid gas from the reducing hydrogen by chemical 40 absorption methods in water or basic solutions were entirely unsuited to the regeneration of the reductant gas. The reason for this was traced to the fact that chromium chloride has a very low tolerance for water vapor or any oxygen containing gas in fact. Thus, for example, I found that the reaction



permits at 800° C. of a partial pressure of H<sub>2</sub>O of 50 only  $1.5 \times 10^{-6}$  atmospheres when the pressure of HCl is 1 atmosphere, but under conditions permitting the continuous reduction of CrCl<sub>2</sub>, corresponding to 3.12% HCl, the tolerance drops and is only

$$(1.5 \times 10^{-6}) \times (0.0312)^2 = 1.5 \times 10^{-9} (\text{approx.})$$

as the partial pressure of water vapor in atmospheres. Any amount of water vapor in excess of this is completely reacted to chromium trioxide. 60 Similarly, I found the tolerance of CrCl<sub>2</sub>, corresponding to the reaction



is a partial pressure of water vapor of  $4.5 \times 10^{-5}$  atmospheres, at 800° C., when the partial pressure 65 of hydrochloric acid is 0.0312 atm. and hydrogen is practically 1 atmosphere.

Finally, in the case of chromium metal itself, I found the tolerance corresponding to the reaction 70 2Cr+3H<sub>2</sub>O=Cr<sub>2</sub>O<sub>3</sub>+3H<sub>2</sub> is  $2.7 \times 10^{-7}$  atmospheres partial pressure of water vapor at 800° C. when the hydrogen is near one atmosphere.

From the above it is clear that the impurities in commercial hydrogen, including oxygen from a 75

few hundredths to 0.5%, or the water vapor left by such excellent drying agents as concentrated sulphuric acid, calcium chloride, etc., are more than sufficient to cause serious oxide contamination when used to prepare the hydrogen for reduction of  $\text{CrCl}_3$ .

*Manner of practicing the invention*

I have discovered a presently related method of 10 eliminating these difficulties successfully with respect to hydrogen and of setting up a continuous reduction and purification which produces substantially chemically pure sponge chromium which contains less than about 0.5% of oxide, 15 with traces only of iron and carbon.

The manner in which the invention is preferably practiced will be best disclosed and understood by reference to the drawing, wherein the 20 single figure is a flow sheet indicating in a schematic manner the process of the present invention.

Commercial hydrogen is first purified of oxygen as by passing it through a drier 3, then over a nickel catalyst 4 at about  $600^\circ \text{C}$ ., and again over 25 a drier 5, and thence passes into storage container 6, where it is stored over a dehydrating agent as concentrated sulphuric acid. (Suitable valves, pressure regulating devices, temperature and pressure indicating devices, are included in the 30 operating system but are not shown.)

The hydrogen storage container 6 is connected to a closed gas circulating system consisting of a pair of sorption purifiers 7 and 8 containing active 35 carbon, a circulating pump 9, a final purifier 10 containing active carbon, and the reducing furnace 11. The first sorption purifiers 7 and 8 are operated at ordinary temperatures, alternately. It has been found that commercial grades of 40 active carbon are capable of preferentially absorbing hydrochloric acid gas up to 4 to 5% of the weight of carbon under these conditions, before appreciable HCl passes through an absorber unadsorbed. When this point is reached, the alternate absorber is connected in the circulating 45 system, and the saturated one is desorbed by first heating to about  $200^\circ \text{C}$ ., which drives off approximately 80% of the retained HCl, after which the temperature is further raised to about  $300^\circ \text{C}$ ., and the purifier is flushed with about 10% of the 50 volume of gas which has been purified during the previous half cycle, using fresh hydrogen, admitted through line 12 from the storage container 6. This removes the remainder of the adsorbed 55 HCl and water vapor. It is then ready for further use. The HCl is driven off and absorbed in water or any desired material suitable for the preparation of a commercial by-product in the absorber 16.

After leaving the pump, and before actually entering the reduction furnace, the gas is given a final purification in adsorber 10 containing active carbon and cooled to  $-70$  to  $-40^\circ$  with carbon dioxide snow. Small amounts of water vapor 60 passing the larger absorbers (which are essentially the HCl adsorbers) are thus virtually completely removed. The regeneration of the accessory purifier need be accomplished only after relatively long periods of operation, since the amount of 65 material retained is small. The regeneration is carried out in a manner similar to the larger units.

The reduction unit is an electric tube furnace 11 of square or rectangular cross section through 70 which trays containing  $\text{CrCl}_3$  crystals are passed

countercurrent to the flow of hydrogen gas, the maximum temperature being  $802^\circ \text{C}$ . The gases in the furnace are not corrosive to ordinary steel, and the tube of the furnace may be either steel protected on the outside from oxidation by air, or 5 of a non-scaling chrome-nickel steel. An especially satisfactory type of construction is to provide a double walled tube, the outer wall 21 being chrome nickel steel, and the inner wall 22 of ordinary low carbon steel. Hydrogen from line 10 23 is admitted to the space between the walls and is maintained at slightly above 1 atmosphere pressure. This permits the use of either a single, or multiple assembly of inner ducts, which may be made of low carbon steel of light gauge, and 15 which are readily replaceable. This construction eliminates transfusion of gases through the furnace walls which might be deleterious to the reducing action.

For introducing and removing trays from the 20 furnace without contamination of the reducing gas, suitable gas locks 26 and 27 are placed at the inlet and outlet end of the furnace. These are operated in the usual manner, being purged and 25 filled with hydrogen from lines 28 and 29 to ensure preservation of the oxygen free atmosphere in the furnace.

I have found that, while normally the reduction takes place in steps, first to  $\text{CrCl}_2$  and later to 30 metal, resulting in concentrations near 4.7% HCl maximum when using the continuous countercurrent apparatus, that, by using high gas velocities and causing the trays to enter rapidly the  $800^\circ$  zone of the furnace, I am able to obtain an 35 exit gas as high as 8 to 10% HCl. This may be interpreted as showing that to some extent direct reduction of  $\text{CrCl}_3$  to metal is in part attained. I have also obtained hydrochloric acid concentrations 40 above the  $\text{CrCl}_2-\text{H}_2-\text{Cr}-\text{HCl}$  limit when using slow gas rates and slow rates of tray admission, but in this case the result was presumably due to a preponderance of the reaction.



My invention is applicable to the reduction of 45 either of the solid chromium chlorides, whether stepwise or direct, and may obviously also be utilized for producing anhydrous chromium chloride, since the formation of metallic chromium 50 can be completely prevented at low gas rates by maintaining the entrant hydrogen with a content of HCl of at least 3.12%.

In practicing my invention, it is desirable to 55 remove all traces of moisture which may be contained on or in the chromium chloride. The so-called violet anhydrous crystals of  $\text{CrCl}_3$ , which are virtually insoluble in water, nevertheless are capable of adsorbing several percent water when they have previously contacted this medium as liquid, or been stored in air of normal humidity. I have found it desirable, therefore, to dry the 60 crystals by heating them, preferably to  $200^\circ-300^\circ \text{C}$ . and preferably in a vacuum, before introducing them into the reduction furnace, and to carry 65 out the transfer quickly, or in a dried atmosphere, so that recontamination is avoided. Temperatures higher than this must not be used not only because the chloride vaporizes and dissociates, but also because the crystals become reactive with 70 oxygen at temperatures slightly above  $300^\circ \text{C}$ . This step is indicated at 31.

Thus it is seen that while one patentee found it necessary to utilize temperatures above  $1600^\circ \text{C}$ . to reduce chromium successfully by hydrogen, by 75

carrying on the reduction from the  $\text{CrCl}_3$  form under the conditions, and in the manner specified above, I have been able to produce chromium in the true sponge form at temperatures of  $800^\circ \text{ C}$ . and in a continuous counter-current unit, and have demonstrated the feasibility of producing a new form of chromium having metallurgical advantages. The new product, sponge chromium, is claimed in a companion application, Serial No. 10 157,153 of even date.

I claim:

1. A process for the reduction of a chromium chloride to chromium comprising reducing said chloride with substantially only dry hydrogen at a temperature of about  $775^\circ \text{ C}$ . in a reducing zone.
2. A process for reduction of a chromium chloride to chromium comprising reducing said chloride with substantially dry pure hydrogen at a temperature of  $775^\circ$ – $850^\circ \text{ C}$ . in a reducing zone,
- 20 removing hydrogen containing hydrogen chloride from the reducing zone and separating hydrogen chloride and water vapor therefrom by a treatment including passage of the hydrogen over activated carbon, and returning the purified hydrogen to the reducing zone.
- 25 3. A process for the reduction of a chromium chloride to chromium comprising reducing said chloride with substantially dry hydrogen at a temperature of about  $775^\circ \text{ C}$ . in a reducing zone,
- 30 removing hydrogen containing  $\text{HCl}$  from the reducing zone, separating  $\text{HCl}$  and water vapor from said removed hydrogen by contacting said removed hydrogen with activated carbon, and returning the purified hydrogen to the reducing zone.
- 35 4. In a process of reducing a chromium chloride to chromium, the step of passing substantially dry pure hydrogen counter-current to said chloride in a reduction zone in a furnace at about  $800^\circ \text{ C}$ . at such a rate that hydrogen leaving said furnace carries about 4.7%  $\text{HCl}$ .
- 40 5. In a process of reducing chromium trichloride to chromium dichloride, the step of passing substantially dry oxygen free hydrogen containing about 3.12%  $\text{HCl}$  over said trichloride chloride in a reduction zone at a temperature of about  $802^\circ \text{ C}$ .
- 45 6. In a process of reducing chromium trichloride to chromium dichloride, the step of passing substantially dry oxygen free hydrogen containing a small amount of  $\text{HCl}$  over said chloride in a reduction zone at a temperature between  $775^\circ$ – $802^\circ \text{ C}$ .
- 50 7. A reduction process comprising heating only substantially dry chromium trichloride to a temperature of  $775^\circ$ – $850^\circ \text{ C}$ . and passing thereover and into direct contact therewith substantially dry pure hydrogen to reduce said chloride entirely to chromium.
- 55 8. A reduction process comprising heating only substantially dry chromium trichloride to a temperature at which hydrogen reduces said chloride to chromium and at which substantial volatilization is absent and passing thereover and into direct contact therewith substantially dry pure hydrogen.
- 60 9. A process for the production of sponge chromium comprising heating substantially dry chro-

mium trichloride to a temperature of  $775^\circ$ – $802^\circ \text{ C}$ . and passing dry pure hydrogen thereover to reduce said chloride to a chromium macroscopically pseudomorphic with said chloride and substantially free of grain growth.

10. Reducing chromic chloride to chrome by passing dry hydrogen over a mass consisting of substantially only said chloride at a temperature between  $775^\circ$  and  $802^\circ \text{ C}$ . to reduce said chromic chloride directly to chromium, and continuing to pass said hydrogen until said mass consists substantially only of chrome.

11. Reducing chromic chloride to chrome by passing dry hydrogen over a mass consisting of substantially only said chloride at a temperature between  $775^\circ$  and  $815^\circ \text{ C}$ . to reduce said chromic chloride directly to chromium, and continuing to pass said hydrogen until said mass consists substantially only of chrome.

12. Reducing chromic chloride to chrome by passing dry hydrogen over a mass consisting of substantially only said chloride at a temperature between  $775^\circ$  and  $850^\circ \text{ C}$ . to reduce said chromic chloride directly to chromium, and continuing to pass said hydrogen until said mass consists substantially only of chrome.

13. Reducing chromic chloride to chrome by passing dry hydrogen containing less than 4.7%  $\text{HCl}$  over a mass consisting of substantially only said chloride at a temperature between  $775^\circ$  and  $802^\circ \text{ C}$ . to reduce said chromic chloride directly to chromium, and continuing to pass said hydrogen until said mass consists substantially only of chrome.

14. Reducing chromic chloride to chrome by passing dry hydrogen containing less than 4.7%  $\text{HCl}$  over a mass consisting of substantially only said chloride at a temperature between  $775^\circ$  and  $815^\circ \text{ C}$ . to reduce said chromic chloride directly to chromium, and continuing to pass said hydrogen until said mass consists substantially only of chrome.

15. Reducing chromic chloride to chrome by passing dry hydrogen containing less than 4.7%  $\text{HCl}$  over a mass consisting of substantially only said chloride at a temperature between  $775^\circ$  and  $850^\circ \text{ C}$ . to reduce said chromic chloride directly to chromium, and continuing to pass said hydrogen until said mass consists substantially only of chrome.

16. In a process of reducing chromium trichloride with hydrogen to chrome metal whereby a hydrogen effluent stream containing about 5% hydrogen chloride is produced, the steps of passing said effluent stream into contact with activated carbon to remove said hydrogen chloride substantially entirely and simultaneously maintain the water content thereof at a point whereat the partial pressure of water vapor in the hydrogen is less than about  $4.5 \times 10^{-5}$  atmospheres, at a temperature of about  $800^\circ \text{ C}$ .

17. In a process of reducing chromium trichloride to chrome metal utilizing hydrogen as the reductant, the steps which consist in employing as feed material chromium trichloride containing less than 0.05% water while maintaining the reduction temperature between  $775^\circ$  and  $850^\circ \text{ C}$ .

CHARLES G. MAIER.